

1

3,752,674

**SILVER HALIDE EMULSION FOGGED WITH A BORON HYDRIDE AND A GOLD COMPOUND**

William Arthur Pritchett, Jr., Rochester, N.Y., assignor to E. I. du Pont de Nemours and Company, Wilmington, Del.

No Drawing. Filed June 22, 1971, Ser. No. 155,629

Int. Cl. G03c 1/28

U.S. CL. 96—108

12 Claims

**ABSTRACT OF THE DISCLOSURE**

Direct-positive photographic elements of high speed and maximum density are prepared by incorporating in the silver halide emulsion at least one boron hydride containing from 6 to 12 boron atoms in which the skeletal framework forms a polyhedron or a fragment thereof, and which may contain heteroskeletal atoms selected from the group consisting of carbon, sulfur and nitrogen, and a gold compound.

**BACKGROUND OF THE INVENTION**

This invention relates to direct-positive colloid-silver halide emulsions. Most particularly it relates to such emulsions which are prefogged by a synergistic combination of chemical fogging agents.

**PRIOR ART**

Direct-positive emulsions are, of course, well known and there are many different methods of producing direct positive images. For example, a silver halide emulsion may be given a short overall exposure of high intensity radiation and then given a longer imagewise exposure of lower intensity. Upon development, a direct positive image will be obtained. Another method is to expose imagewise and develop and bleach-out developed silver and then flash expose and redevelop. A still further method is to use emulsion coated elements which have been chemically fogged with, for example, formaldehyde, hydrazine, sodium arsenite, silver ions and other fogging agents such as gold salts and sulfur compounds. Combinations of the above compounds such as hydrazine and gold salts have also been suggested. Upon imagewise exposure and development of such chemically fogged elements, a positive image is obtained directly. In direct positive photographic elements utilizing this latter method, there is usually incorporated a desensitizing compound, usually a colored desensitizing dye.

The prior systems have some shortcomings in terms of speed, contrast and other sensitometric characteristics. When using a sufficient quantity of reducing agent, e.g., stannous chloride, the fogged silver halide grains cannot be easily bleached so that excessively long exposure is required and clean backgrounds or low minimum densities cannot be obtained. When gold compounds are used alone, difficulties are again experienced in obtaining sufficiently fogged grains and, as in the case of stannous chloride, the fogged grains are not easily bleached without impractically long exposures. It has been proposed to increase the speed of the above systems by adding certain dyes but, in many cases, this causes undesirable stain. A significant improvement resulted from the use of amine boranes as chemical fogging agents in direct positive emulsion systems. Direct positive emulsions and elements comprising such emulsions are described and claimed in U.S. patents Bigelow and Burt, 3,361,564, Jan. 2, 1968 and Burt, 3,445,235, May 10, 1969. Overman 3,655,390, Apr. 11, 1972 and Burt 3,607,288, Sept. 21, 1971. U.S. 3,445,235 discloses and claims the use of rhodium and iridium salts in the direct positive emulsions of Bigelow

2

et al. 3,361,564 and the Overman patent discloses the use of bismuth as antikinking agents. U.S. 3,607,288 discloses the use of gold salts in direct positive emulsions chemically fogged with amine boranes to reduce the tendency for red light to bleach the fogged layer. Further improvements were made in shelf life or aging stability and contrast of direct positive elements by use of boron hydrides in which a skeletal framework forms a polyhedron or fragment thereof, and which may contain heteroskeletal atoms selected from the group consisting of carbon, sulfur and nitrogen. The compounds are added in quantities ranging up to  $2.4 \times 10^{-4}$  mole per 1.5 moles of silver under pH conditions of 3.0 to 9.0. Direct positive elements comprising such emulsions are described and claimed in assignee's Bigelow, U.S. Patent 3,637,392, Jan. 25, 1972. Compared to a typical commercial film of the prior art which are chemically fogged with e.g., formaldehyde, the speed, of which, in terms of  $100/E \times 10^{-6}$ , is about 109, the direct positive elements containing the borane compound have speeds ranging from 126 to 14,000.

**SUMMARY OF THE INVENTION**

It has now been found that improved high quality direct positive silver halide emulsions, speed and contrast can be obtained by the use of a synergistic combination of (1) at least one boron hydride in which the skeletal framework forms a polyhedron or fragment thereof containing from 6 to 12 boron atoms and may contain heteroskeletal atoms selected from the group consisting of carbon, sulfur and nitrogen atoms and (2) a gold compound. The boron hydride or cyclic boranes may be added in the range of  $10^{-8}$  to  $10^{-6}$  mole per mole of silver and the gold compound which may be a water-soluble salt or an acid such as hydrochloroauric acid may be added in the range of  $10^{-6}$  to  $10^{-3}$  mole per mole of silver nitrate. The synergistic combination of borane and gold compounds may be added to the emulsion at a pH  $\leq 9.0$ . The borane compounds may be added as a solution with a suitable solvent, i.e., water, ethyl alcohol, benzene, acetone, dioxane, etc. The useful borane compounds in aqueous solutions have greater stability than the amine boranes of the above Bigelow and Burt and Burt patents.

**PREFERRED EMBODIMENT**

The effectiveness of some borane compounds of Bigelow, U.S. Pat. 3,637,392 in fogging a silver halide emulsion is not affected by the pH of the systems and they show good fogging properties under acid as well as alkaline conditions. Certain borane compounds are more effective than others when used in equivalent quantities. According to this invention it is important that the borane and gold compounds be added at the beginning, during or before the end of the digestion period after the excess salts have been removed by washing. The pH of the system can be adjusted to 9.0 or below and preferably is adjusted to 7.0 or below. The fogging effect produced by the borane compound/gold ion combination is bleachable by light prior to development. The emulsions of the invention may also contain rhodium or iridium in an amount of 1.5 to 325 mg. of a salt of such elements per mole of silver. Suitable salts are described in U.S. Pat. 3,445,235.

Suitable developers are conventional, alkaline, photographic developing solutions useful for standard direct positive emulsions in the absence of the novel fogging combination. While the silver halide system used in this invention is generally a silver chlorobromide, other types, e.g., silver chloride, silver iodobromide, silver iodochloride and silver iodobromochloride, may be used with the boron hydride/gold compound combination.

Among the borane compounds which have been found useful in the fogging composition of this invention are the homonuclear boranes, polyheteronuclear boranes comprising polyhedral azoboranes, polyhedral thiaboranes and polyhedral carboranes, representative examples of which are shown in the following list.

## COMPOUND

$(\text{NH}_4)_2\text{B}_{10}\text{H}_{10}$   
 $\text{CsB}_9\text{H}_{12}\text{S}$   
 $(\text{CH}_3)_3\text{NNB}_9\text{H}_{12}$   
 $(\text{CH}_3)_4\text{N}(\text{CH}_3)_2\text{NNB}_9\text{H}_{12}$   
 $[(\text{C}_6\text{H}_5)_3\text{CH}_3\text{P}]_2\text{B}_{11}\text{H}_{11}$   
 $\text{B}_{10}\text{H}_{10}\text{CNH}_3$   
 $(\text{CH}_3)_4\text{N}(\text{CH}_3)_2\text{CNHCB}_{10}\text{H}_{12}$   
 $(\text{CH}_3)_3\text{NHB}_{10}\text{H}_{12}\text{CH}$   
 $\text{B}_{10}\text{H}_{12}[\text{S}(\text{CH}_3)_2]_2$   
 $\text{B}_9\text{H}_{13}\text{S}(\text{C}_2\text{H}_5)_2$   
 $\text{B}_{10}\text{H}_{12}[\text{S}(\text{C}_2\text{H}_5)_2]_2$   
 $\text{C}_6\text{H}_5\text{B}_{11}\text{H}_{10}\text{S}$   
 $\text{Na}_2\text{B}_{12}\text{H}_{12}\cdot 2\text{H}_2\text{O}$   
 $\text{B}_{10}\text{C}_2\text{H}_{12}$   
 $\text{Cs}(\text{CH}_3)_4\text{NB}_{11}\text{H}_{11}$   
 $\text{Cs}_2\text{B}_8\text{H}_6$   
 $\text{CsB}_9\text{H}_9\text{CH}$

Methods of preparation of these compounds may be found in The Chemistry of Boron and its Compounds, E. L. Meutterties, John Wiley and Sons, N.Y., 1967; Polyhedral Boranes, E. L. Meutterties and W. H. Knoth, Marcel Dekker, Inc., N.Y. 1968, and numerous patents by these authors.

Among the gold compounds which will be found useful, there may be mentioned hydrochloroauric acid, auric chloride, auric bromide, sodium and potassium aurate, sodium and potassium chloroaurate, bromoaurate and iodoaurate, potassium auricyanide and potassium aurithiocyanate.

For the most efficient effect, it is preferred that the borane compounds and gold compounds be added to the silver halide emulsion after it has been made, ripened and washed to remove the excess soluble salts resulting from the precipitation of the silver halides and after the pH has been adjusted to  $\leq 9.0$  and preferably between 3 and 7.0. The preselected level of pH should be maintained during the digestion period. After digestion, the pH is adjusted to the desired coating pH and the conventional final adjuvants are incorporated with the emulsion. Coating aids such as saponin, sodium salts of polyether sulfonates, long chain alkyl sulfonates and sulfates, cetyl betaine, etc., can be utilized. The emulsion is then coated onto a suitable support and dried. The conventional coating processes and apparatus can be used.

The sensitometric characteristics of the direct positive elements may be determined by exposing in an intensity scale sensitometer, described on page 616, Mees, The Theory of the Photographic Process, Macmillan Company, New York (1942), using a suitable step wedge and light intensity depending upon the inherent speed of the emulsion. After exposure in the sensitometer, the strips are developed in suitable developers as shown below, immersed in a short-stop bath, fixed in a conventional fixing solution, and then washed and dried.

In evaluating the processed strips, the maximum density is the highest density on the step wedge. The speed of a typical low speed commercial direct positive in terms of  $100/\text{E} \times 10^{-6}$  is 103 and the conventional material has a  $D_{\text{max}}$  of about 3.5.

The invention will now be illustrated in and by the following examples:

## EXAMPLE 1

10 A direct positive emulsion was made in the following manner. To acidified aqueous solutions of gelatin each containing 1 mole of  $\text{KCl}$  and  $6.8 \times 10^{-5}$  mole of  $\text{RhCl}_3$ , there were rapidly added solutions containing 1 mole of  $\text{AgNO}_3$ . To each of the resulting mixtures there was added 15 0.4 mole of  $\text{KBr}$  in aqueous solution and the emulsions were then ripened by heating for 10 minutes at  $160^\circ \text{ F}$ . A second quantity of 0.6 mole of  $\text{KBr}$  in aqueous solution was added to each and the emulsions were again ripened for 10 minutes at  $160^\circ \text{ F}$ .

20 The resulting silver bromochloride emulsions were then coagulated, washed and redispersed in the manner disclosed in Moede, U.S. Patent 2,772,162, Nov. 27, 1956. The temperature of the redispersed emulsion was raised to  $130^\circ \text{ F}$ . and there was added an aqueous solution containing 6.1% gelatin. The pH was adjusted to 5.5 using 0.6 M  $\text{NaOH}$ . The borane compound,  $\text{CsB}_9\text{H}_{12}\text{S}$  was added to each emulsion as shown in the table below and then a solution of hydrochloroauric acid ( $\text{HAuCl}_4$ ) was added in quantities shown in the tables and then the emulsion was digested at  $130^\circ \text{ F}$ . for 40 minutes. The emulsion temperature was then reduced to  $90^\circ \text{ F}$ . and 6 grams of poly(ethyl acrylate) as a 32% solids solution was added along with the usual coating aids including a gelatin hardener. The emulsions were coated on a photographic film support and dried in a conventional manner. Strips of the exposed emulsion elements were exposed in the above described sensitometer and processed in the following manner using a  $\sqrt{2}$  step and a log exposure 4.25. A coated test strip was exposed and developed for  $1\frac{1}{2}$  minutes at  $68^\circ \text{ F}$ . in a developer having the following composition:

Water—750 ml.  
 Methyl-p-aminophenol sulfate—3.0 grams  
 45 Sodium bisulfite—1.6 grams  
 Sodium sulfite (anhydrous)—45.0 grams  
 Hydroquinone—12.0 grams  
 Sodium carbonate (anhydrous)—67.5 grams  
 Potassium bromide—1.9 grams  
 50 Trisodium ethylene diamine tetra acetate trihydrate—  
 1.0 gram  
 Benzotriazole—0.25 gram  
 Water to make—1.0 liter

55 The strip was then immersed in a conventional short stop for 5–10 seconds, fixed for three minutes in a conventional fixer, then washed and dried.

In evaluation of the processed strips, the minimum density ( $D_{\text{min.}}$ ) equals the lowest density above that of the fixed out strip mentioned above. The maximum density ( $D_{\text{max.}}$ ) is the highest density above  $D_{\text{min.}}$ ) Gamma ( $\gamma$ ), the slope of the characteristic H&D curve is determined in the usual manner. Sensitometric results are shown in Tables I and IA.

TABLE I

| Mole<br>$\text{CsB}_9\text{H}_{12}\text{S}/$<br>mole $\text{AgNO}_3$ | Mole<br>$\text{HAuCl}_4 \cdot 3\text{H}_2\text{O}/$<br>mole $\text{AgNO}_3$ | Speed,<br>$100/\text{E} \times 10^{-6}$ | $D_{\text{max.}}$ | $D_{\text{min.}}$ | Gamma |
|----------------------------------------------------------------------|-----------------------------------------------------------------------------|-----------------------------------------|-------------------|-------------------|-------|
| $13.3 \times 10^{-8}$                                                | 0                                                                           | —                                       | —                 | —                 | —     |
| $26.6 \times 10^{-8}$                                                | 0                                                                           | —                                       | —                 | —                 | —     |
| $53.2 \times 10^{-8}$                                                | 0                                                                           | —                                       | 0.19              | —                 | —     |
| $106.4 \times 10^{-8}$                                               | 0                                                                           | —                                       | 0.62              | 0.32              | —     |
| 0                                                                    | $4.96 \times 10^{-4}$                                                       | —                                       | —                 | —                 | —     |
| $13.3 \times 10^{-8}$                                                | $4.96 \times 10^{-4}$                                                       | 689,000                                 | 3.15              | 0.04              | 1.06  |
| $26.6 \times 10^{-8}$                                                | $4.96 \times 10^{-4}$                                                       | 364,000                                 | 3.49              | 0.05              | .86   |
| $39.9 \times 10^{-8}$                                                | $4.96 \times 10^{-4}$                                                       | 321,000                                 | 3.52              | 0.05              | 1.06  |
| $53.2 \times 10^{-8}$                                                | $4.96 \times 10^{-4}$                                                       | 77,000                                  | 4.30              | 0.11              | 1.13  |
| $79.8 \times 10^{-8}$                                                | $4.96 \times 10^{-4}$                                                       | 85,000                                  | 5.16              | 0.13              | 0.93  |

TABLE IA

| Mole<br>(NH <sub>4</sub> ) <sub>2</sub> B <sub>10</sub> H <sub>10</sub> /<br>mole AgNO <sub>3</sub> | Mole<br>HAuCl <sub>4</sub> ·3H <sub>2</sub> O/<br>mole AgNO <sub>3</sub> | Speed,<br>100/E × 10 <sup>-4</sup> | D <sub>max.</sub> | D <sub>min.</sub> | Gamma |
|-----------------------------------------------------------------------------------------------------|--------------------------------------------------------------------------|------------------------------------|-------------------|-------------------|-------|
| 1.00 × 10 <sup>-4</sup>                                                                             | 0                                                                        |                                    |                   |                   |       |
| 2.66 × 10 <sup>-4</sup>                                                                             | 0                                                                        |                                    |                   |                   |       |
| 6.68 × 10 <sup>-5</sup>                                                                             | 0                                                                        |                                    |                   |                   |       |
| 0                                                                                                   | 1.02 × 10 <sup>-5</sup>                                                  |                                    |                   |                   |       |
| 6.68 × 10 <sup>-5</sup>                                                                             | 1.02 × 10 <sup>-5</sup>                                                  | 725,000                            | 0.81              | 0.06              | 0.9   |
| 13.30 × 10 <sup>-5</sup>                                                                            | 1.02 × 10 <sup>-5</sup>                                                  | 550,000                            | 1.47              | 0.09              | 1.1   |
| 20.0 × 10 <sup>-5</sup>                                                                             | 1.02 × 10 <sup>-5</sup>                                                  | 221,000                            | 3.05              | 0.12              | 1.6   |
| 26.6 × 10 <sup>-5</sup>                                                                             | 1.02 × 10 <sup>-5</sup>                                                  | 153,000                            | 3.63              | 0.11              | 3.0   |

## EXAMPLE II

To an aqueous gelatin solution containing 7.95 milligrams of RhCl<sub>3</sub> there was added by a twin-stream method over a 90-second period, 1 mole of AgNO<sub>3</sub> and 1 mole of KBr in aqueous solutions. The resulting emulsion was then ripened by heating with 0.73 mole of aqueous NH<sub>4</sub>OH for 10 minutes at 110° F. The emulsion was coagulated, washed and redispersed as described in Moede, U.S. 2,772,165, issued Nov. 27, 1956. The redispersed emulsion was added to an aqueous solution containing 6.1% gelatin and heated to 130° F. with the pH being adjusted to 5.5 with 0.6 M NaOH. The borane compound, (NH<sub>4</sub>)<sub>2</sub>B<sub>10</sub>H<sub>10</sub> was added as indicated in the table below followed by the addition of HAuCl<sub>4</sub>, hydrochlorauric acid as indicated.

The emulsion was digested for 40 minutes at 130° F. The temperature was reduced to 90° F. and 6 grams of poly(ethyl acrylate) as a 32% solids solution was added along with the usual coating aids including a gelatin hardener. The emulsion was then coated on a photographic film support and dried in a conventional manner. Strips of

AgNO<sub>3</sub>. Upon completion of the silver halide precipitation, the composition of the emulsion was about 60% bromide and 40% chloride. The pH was adjusted to 3.9, the emulsion was coagulated, washed and redispersed as described in Example I. The redispersed emulsion is added to an aqueous solution containing 6.1% gelatin and heated to a temperature of 130° F. The pH of the system was adjusted to 5.5 ± 0.5 with 0.6 M NaOH. An aqueous solution of the cyclic borane compound CsB<sub>9</sub>H<sub>12</sub>S was added to portions of the emulsion as indicated in the table below together with HAuCl<sub>4</sub> as shown. The emulsions were digested at 130° F. for 40 minutes. The emulsion temperature was reduced to 90° F. and poly(ethyl acrylate) as a 32% solids solution was added along with the conventional coating aids including a gelatin hardener. The emulsions were coated on a photographic film support and dried in a conventional manner.

Strips of the films were exposed and processed as described in Example I. Sensitometric data are shown in the following table.

TABLE III

| Mole<br>CsB <sub>9</sub> H <sub>12</sub> S/<br>mole AgNO <sub>3</sub> | Mole<br>HAuCl <sub>4</sub> ·3H <sub>2</sub> O/<br>mole AgNO <sub>3</sub> | Speed,<br>100/E × 10 <sup>-4</sup> | D <sub>max.</sub> | D <sub>min.</sub> | Gamma |
|-----------------------------------------------------------------------|--------------------------------------------------------------------------|------------------------------------|-------------------|-------------------|-------|
| 0                                                                     | 2.46 × 10 <sup>-4</sup>                                                  | 0                                  | 0                 | 0                 | 0     |
| 2.4 × 10 <sup>-5</sup>                                                | 0                                                                        | 12,300                             | 3.49              | 0                 | ----- |
| 9.3 × 10 <sup>-5</sup>                                                | 0                                                                        | 0                                  | 0                 | 0                 | 0     |
| 9.3 × 10 <sup>-5</sup>                                                | 2.46 × 10 <sup>-4</sup>                                                  | 243,000                            | 2.35              | 0.04              | 1.11  |

the coatings were exposed and processed as described in Example I. Sensitometric data is shown below.

TABLE II

| Mole<br>(NH <sub>4</sub> ) <sub>2</sub> B <sub>10</sub> H <sub>10</sub> /<br>mole AgNO <sub>3</sub> | Mole<br>HAuCl <sub>4</sub> ·3H <sub>2</sub> O/<br>mole AgNO <sub>3</sub> | Speed,<br>100/E × 10 <sup>-4</sup> | D <sub>max.</sub> | D <sub>min.</sub> | Gamma |
|-----------------------------------------------------------------------------------------------------|--------------------------------------------------------------------------|------------------------------------|-------------------|-------------------|-------|
| 2.66 × 10 <sup>-4</sup>                                                                             | 0                                                                        |                                    |                   |                   |       |
| 0                                                                                                   | 1.02 × 10 <sup>-5</sup>                                                  |                                    |                   |                   |       |
| 2.65 × 10 <sup>-7</sup>                                                                             | 1.02 × 10 <sup>-5</sup>                                                  | 337,000                            | 2.70              | 0.00              | 0.80  |
| 5.30 × 10 <sup>-7</sup>                                                                             | 1.02 × 10 <sup>-5</sup>                                                  | 98,500                             | 3.60              | 0.00              | 0.80  |
| 7.90 × 10 <sup>-7</sup>                                                                             | 1.02 × 10 <sup>-5</sup>                                                  | 47,500                             | 4.32              | 0.00              | 0.73  |
| 10.60 × 10 <sup>-7</sup>                                                                            | 1.02 × 10 <sup>-5</sup>                                                  | 47,500                             | 4.43              | 0.00              | 0.80  |

## EXAMPLE III

To an aqueous gelatin solution containing 31.8 milligrams of RhCl<sub>3</sub> there was added simultaneously by the twin stream method over a period of about 200 seconds, 60 a salt solution containing 0.6 mole KBr and 1.3 moles of KCl and an aqueous solution containing 1 mole of

## EXAMPLE IV

Example I was repeated using the quantities of hydrochlorauric acid and the various borane compounds as indicated in the table below. The pH of the emulsions were maintained at 7.0 during the digestion period. Exposure, development and evaluation of sensitometric data was carried out as indicated in Example I.

TABLE IV

| Borane compound,<br>mole/mole AgNO <sub>3</sub>                                                                                         | Mole<br>HAuCl <sub>4</sub> ·3H <sub>2</sub> O/<br>mole AgNO <sub>3</sub> | Speed 100/E<br>× 10 <sup>-4</sup> | D <sub>max.</sub> | D <sub>min.</sub> |
|-----------------------------------------------------------------------------------------------------------------------------------------|--------------------------------------------------------------------------|-----------------------------------|-------------------|-------------------|
| CsB <sub>9</sub> H <sub>12</sub> S, 2.66 × 10 <sup>-7</sup>                                                                             | 0                                                                        | 0                                 | 0                 | 0                 |
| CsB <sub>9</sub> H <sub>12</sub> S, 2.66 × 10 <sup>-7</sup>                                                                             | 4.95 × 10 <sup>-5</sup>                                                  | 280,000                           | 1.37              | 0.05              |
| [(C <sub>4</sub> H <sub>9</sub> ) <sub>2</sub> CH <sub>2</sub> ] <sub>2</sub> Pb <sub>2</sub> H <sub>11</sub> , 2.66 × 10 <sup>-7</sup> | 0                                                                        | 0                                 | 0                 | 0.03              |
| [(C <sub>4</sub> H <sub>9</sub> ) <sub>2</sub> CH <sub>2</sub> ] <sub>2</sub> Pb <sub>2</sub> H <sub>11</sub> , 2.66 × 10 <sup>-7</sup> | 4.95 × 10 <sup>-5</sup>                                                  | 243,000                           | 1.83              | 0.05              |
| B <sub>10</sub> C <sub>2</sub> H <sub>12</sub> , 6.68 × 10 <sup>-7</sup>                                                                | 4.95 × 10 <sup>-5</sup>                                                  | 168,000                           | 1.16              | 0.05              |
| Cs(C <sub>2</sub> H <sub>5</sub> ) <sub>4</sub> NB <sub>11</sub> H <sub>11</sub> , 6.68 × 10 <sup>-7</sup>                              | 4.95 × 10 <sup>-5</sup>                                                  | 350,000                           | 1.00              | 0.05              |
| Cs <sub>2</sub> B <sub>6</sub> H <sub>6</sub> , 2.66 × 10 <sup>-7</sup>                                                                 | 4.95 × 10 <sup>-5</sup>                                                  | 102,000                           | 4.27              | 0.05              |
| Cs <sub>2</sub> B <sub>6</sub> H <sub>6</sub> , 2.66 × 10 <sup>-7</sup>                                                                 | 4.95 × 10 <sup>-5</sup>                                                  | 310,000                           | 1.02              | 0.05              |
| Cs <sub>2</sub> B <sub>6</sub> H <sub>6</sub> CH <sub>3</sub> , 2.66 × 10 <sup>-7</sup>                                                 | 4.95 × 10 <sup>-5</sup>                                                  | 49,400                            | 4.91              | 0.05              |
| Cs <sub>2</sub> B <sub>6</sub> H <sub>6</sub> CH <sub>3</sub> , 2.66 × 10 <sup>-7</sup>                                                 | 4.95 × 10 <sup>-5</sup>                                                  | 366,000                           | .74               | 0.05              |

7  
EXAMPLE V

A number of emulsions were prepared as described in Example IV and the borane compound  $(\text{NH}_4)_2\text{B}_{10}\text{H}_{10}$  was used alone and in combination with the borane compound  $\text{CsB}_9\text{H}_{12}\text{S}$  with  $4.95 \times 10^{-5}$  mole  $\text{HAuCl}_4$  per mole of silver nitrate as shown in the table below. Sensitometric data is shown in the table.

TABLE V

| Borane compound                                   | Mole/mole $\text{AgNO}_3$ | Speed     | $D_{\max.}$ | $D_{\min.}$ | Gamma |
|---------------------------------------------------|---------------------------|-----------|-------------|-------------|-------|
| $(\text{NH}_4)_2\text{B}_{10}\text{H}_{10}$ ---   | $2.66 \times 10^{-6}$     | 510,000   | 1.05        | .04         | 0.45  |
| $\text{CsB}_9\text{H}_{12}\text{S}$ -----<br>plus | $2.66 \times 10^{-6}$     | 2,090,000 | 3.61        | .05         | 0.80  |
| $(\text{NH}_4)_2\text{B}_{10}\text{H}_{10}$ ---   | $2.66 \times 10^{-6}$     |           |             |             |       |

As will be seen from the above sensitometric data, the direct positive elements of this invention are extremely fast as compared to the emulsions of the prior art and much faster than when the borane compounds are used in the absence of a gold compound.

From the emulsion coated elements of this invention, good duplicates can be made by contact printing, using suitable exposing radiation. The direct positive elements may be used for reproducing continuous tone negatives, halftones, line copy, engineering drawings, etc. The direct positive elements of this invention may also find use in color photography.

The photographic elements of this invention have the advantage that they provide direct positives with extremely low minimum densities and high maximum densities. They are extremely fast and require much lower quantities of the borane and gold compounds than have been necessary heretofore in the production of chemically fogged direct positive elements. The elements of this invention may be developed in any standard developing solution such as the continuous tone developing solution set forth in Example I above or a high contrast lithographic developer using standard techniques well known in the art. Variations in the developing solution will have much the same effect as would be obtained in developing non-reversal emulsions. No pre-exposure operations or auxiliary processing procedures are necessary or desirable in using the novel elements of this invention. It is also unnecessary to utilize stain producing nonsensitizing dyes or desensitizing dyes although optical sensitizing dyes for extending the range of receptivity of actinic radiation may be incorporated in the system. Further, it is unnecessary to use high quantities of gold compounds which cause poor bleaching characteristics resulting in excess minimum densities or impure white background areas.

In place of gelatin as the water-permeable colloid binder for the silver halide grains as described in the above examples, other natural or synthetic water-permeable organic colloid binding agents can be used. Such agents include water-permeable or water-soluble polyvinyl alcohol and its derivatives, e.g., partially hydrolyzed polyvinyl acetates, polyvinyl ethers, and acetals containing a large number of extra-linear  $-\text{CH}_2\text{CHOH}-$  groups; hydrolyzed interpolymers of vinyl acetate and unsaturated addition polymerizable compounds such as maleic anhydride, acrylic acid and methacrylic acid ethyl esters. Suitable colloids of the last mentioned type are disclosed in U.S. Patents 2,276,322; 2,276,323 and 2,347,811. The useful polyvinyl acetals include polyvinyl butyraldehyde acetal and polyvinyl sodium o-sulfobenzaldehyde acetal. Other useful colloid binding agents include polyvinyl butyraldehyde acetal and polyvinyl sodium o-sulfobenzaldehyde acetal. Other useful colloid binding agents include the poly-N-vinyl lactams of Bolton, U.S. Patent 2,495,918, the hydrophilic copolymers of N-acrylamido alkyl betaines described in Shacklett, U.S. Pat. 2,833,050 and hydrophilic cellulose ethers and esters.

## 8

The emulsions of this invention may be coated on any suitable base including paper and transparent film support. For example, the cellulosic supports, e.g., cellulose acetate, cellulose triacetate, cellulose mixed esters, etc., may be used. Polymerized vinyl compounds, e.g., copolymers of vinyl acetate and vinyl chloride, polystyrene, and polymerized acrylates may also be mentioned. The films formed from polyesters made according to the teachings of Alles, U.S. Patent 2,779,684 and the patents referred to in the specification of that patent. Other suitable supports are the polyethylene terephthalate/isophthalates of British specification No. 766,290 and Canadian Patent 562,672 and those obtainable by condensing terephthalic acid and dimethyl terephthalate with propylene glycol, di-methylene glycol, tetramethylene glycol or cyclohexane-1,4-dimethanol (hexahydro-p-xylene alcohol). The films of Bauer et al., U.S. 3,059,543 may also be used. The polyester films are particularly suitable because of their dimensional stability.

20 The emulsions are generally coated on the supports in quantities to give a coating weight of about 50-75 milligrams of silver halide per square decimeter of support surface area. Other cyclic or polyhedral boranes than those set forth above may be used. A practical limit is imposed 25 upon the use of certain boranes due to high toxicity and possible explosive characteristics of individual compounds.

The embodiments of the invention in which an exclusive property or privilege is claimed are defined as follows:

1. A direct-positive, water-permeable colloid-silver halide emulsion containing a boron hydride and a gold compound, in which the has a polyhedral framework containing from 6-12 boron atoms and may contain heteroskeletal atoms selected from the groups consisting of C, S, and N, wherein, the boron hydride is present in an amount of  $10^{-8}$  to  $10^{-6}$  mole per mole of silver, and the gold compound is present in an amount of  $10^{-6}$  to  $10^{-3}$  mole per mole of silver, the combined amounts of said boron hydride and gold compound being sufficient to fog said emulsion.
2. An emulsion according to claim 1 having pH 3.0-9.0.
3. An emulsion according to claim 1 containing rhodium chloride.
4. An emulsion according to claim 1 wherein the silver halide is a silver chlorobromide emulsion.
5. An emulsion according to claim 1 wherein the silver halide is a silver bromochloride emulsion.
6. An emulsion according to claim 1 wherein the colloid is gelatin.
7. An emulsion according to claim 1 wherein the boron hydride is  $\text{CsB}_9\text{H}_{12}\text{S}$ .
8. An emulsion according to claim 1 wherein the boron hydride is a polyhedral homonuclear borane of the series  $\text{B}_6\text{H}_6^{-2}$  to  $\text{B}_{12}\text{H}_{12}^{-2}$ .
9. An emulsion according to claim 1 wherein the boron hydride is  $(\text{NH}_4)_2\text{B}_{10}\text{H}_{10}$ .
10. An emulsion according to claim 1 wherein the gold compound is hydrochloroauric acid.
11. A photographic element comprising a support bearing a layer of an emulsion as defined in claim 1.
12. A photographic element comprising a support bearing a layer of an emulsion as defined in claim 3.

## References Cited

## UNITED STATES PATENTS

|           |         |              |         |
|-----------|---------|--------------|---------|
| 3,411,917 | 11/1968 | Figueras     | 96-64 X |
| 3,637,392 | 1/1972  | Bigelow      | 96-108  |
| 3,445,235 | 5/1969  | Burt         | 96-95   |
| 3,501,305 | 3/1970  | Illingsworth | 96-108  |

70 NORMAN G. TORCHIN, Primary Examiner  
W. H. LOUIE, JR., Assistant Examiner

U.S. CL. X.R.